

Feb. 24, 1959

B. LÖFGREN ET AL

2,874,481

METHOD OF TREATING FIBRE BOARDS

Filed June 28, 1954

2 Sheets-Sheet 1

FIG. 1.



FIG. 2.



FIG. 3.



FIG. 3a



FIG. 4.



INVENTORS:  
BROR LÖFGREN  
NILS JUL OGLAND

BY *Housten & Housten*  
ATTYS.

Feb. 24, 1959

B. LÖFGREN ET AL

2,874,481

METHOD OF TREATING FIBRE BOARDS

Filed June 28, 1954

2 Sheets-Sheet 2

FIG. 5.



FIG. 6.



TEMPERATURE  
(IN DEGREES CENTIGRADE)



PRESSURE  
(IN ATMOSPHERES)



FIG. 7.

FIG. 8.

INVENTORS:  
BROR LÖFGREN  
NILS JUL ÖGLAND  
BY *Houston & Houston*  
ATTYS.

2,874,481

## METHOD OF TREATING FIBRE BOARDS

Bror Löfgren, Stockholm, and Nils Jul Öglund, Svanskog, Amal, Sweden, assignors to Aktiebolaget Svenska Flaktfabriken, Stockholm, Sweden

Application June 28, 1954, Serial No. 439,848

Claims priority, application Sweden June 29, 1953

6 Claims. (Cl. 34—16)

The present invention relates to an improved method of treating fibre boards and like materials manufactured by defibrating fibrous raw materials. The invention has particular utility in treating materials which have been formed, dehydrated, and dried in a pressing device.

Hard fibrous sheets, such as wall-board are manufactured from cellulose materials such as wood, straw, bagasse, etc. The manufacture is commonly carried out in such a way that the raw material, after having been defibrated, is formed into a web which is then cut into sheets. The sheets are then dehydrated and dried in a pressing device. The pressing is usually performed to produce one smooth surface and one puckered or uneven surface by pressing the sheet between a plane plate and a wire mesh. In certain cases, when manufacturing sheets smooth on both sides, the sheets are bone dried before pressing and are then subjected only to heat and pressure in the pressing device.

In the pressing cycle, the wet sheets are charged into the pressing device and are then exposed to pressure and heat to be dehydrated as the temperature of the sheets is increased. At a certain time, the temperature of the sheets reaches such a value that the sheets are practically bone dry. The sheets are usually allowed to remain in the pressing device until another time, in which period, the sheets are heated under pressure so that they reach a temperature which is almost equal to the temperature of the heated surfaces of the pressing device. In many operations, the procedure is interrupted during this latter period and the sheets are then heat-treated—so called hardening—in a separate device. The reason for this is that the pressing device is an expensive part of the plant, and thus, heat-treating the sheets while in the pressing device would be expensive. The object of the heat treatment is to somewhat increase the strength of the sheets against bending and also to reduce their power of moisture absorption and their swelling due to moisture absorption. The sheets pressed and dried in this way are then moistened to a degree, in order to have their state in equilibrium with the temperature and the relative humidity existing in the place where the sheets are to be used. The prior conventional moistening in moist air is often time-consuming.

The moistening is usually performed by air which is practically saturated with water vapor, and the temperature is maintained at a moderate level, preferably about 35 degrees to 60 degrees C. At high temperatures, the time for moistening decreases because the diffusion of water vapor in the sheet takes place more rapidly at high temperatures than at low temperatures. However, when using high temperatures and a high relative humidity in the air, in order to accelerate the penetrating of the moisture into the sheets, the smoothness of the sheets is spoiled (i. e., the sheet loses part of its lustre). In addition, a so-called "rise" of the fibres occurs in the surface layer of the sheets.

It is an object of the present invention to eliminate

these and other disadvantages of the prior methods of treating hard, wooden fibre sheets, boards or the like.

It is also an object of the invention to improve the quality of the moistened sheets.

5 The invention is mainly characterized in that the material, after having been heat-treated, is charged into the moistening chamber, and the moistening is performed by substantially air-free steam and is followed by cooling. It is possible to use saturated or superheated steam and 10 the steam may be at atmospheric pressure or at super pressure. It is also possible to combine the heat treatment and the moistening of the sheets, and we have found that if this combined heat and moistening treatment is performed under controlled conditions, it is possible to obtain improved results with respect to the decrease in the sheets' power of moisture absorption and their swelling, resulting in a worthwhile increase in the 15 quality of the sheets.

Other objects of the invention will be evident from the 20 claims and the description and with reference to the accompanying drawings wherein:

Fig. 1 is a curve illustrating a conventional pressing cycle;

Fig. 2 is a curve of the hygroscopic properties of fibre-board in an atmosphere of steam, showing the equilibrium relation between the moisture ratio of the sheets and the 25 temperature of the steam at atmospheric pressure;

Figs. 3 and 3a are curves showing cycles of stepwise moistening in accordance with the invention;

Fig. 4 is a curve illustrating a cycle of continuous moistening of sheets in accordance with the invention;

Fig. 5 shows an apparatus for heat-treating or heating and moistening and cooling the sheets in accordance with 30 the invention;

Fig. 6 illustrates apparatus for treating sheets under high pressures in an autoclave in accordance with the 35 invention; and

Figs. 7 and 8 are curves illustrating respectively the 40 variations of the temperature and pressure during a cycle of the treatment in apparatus such as shown in Fig. 6.

When a sheet is moistened in steam according to the 45 invention, the moistening initially has a tendency to proceed very rapidly because of the great difference in vapor pressure which exists between the moistening medium and the sheet. The surface layer of the sheet therefore almost immediately will attain a moisture ratio equal to the equilibrium moisture ratio of the sheet in the steam. The moistening is accompanied by a swelling of the sheet. In accordance with the invention, the moistening is slowed so that moisture from the surface layer has 50 time to penetrate the lower layers to permit these layers to swell to a certain degree. In the present case, it may be assumed that the molecules of water simultaneously penetrate the layers of the fibres both in the center of the sheet and at the surface of the sheet. In a pure atmosphere of water vapor, the air molecules in the sheet compete with the water molecules of the steam within capillary tubes of the sheets. We have found that in spite of this, the moistening proceeds more rapidly in steam than in moist air. At high temperatures, the 55 rapidity of the movement of the molecules is rather great. The water vapor penetrates rapidly into the cavities, because of the high diffusion constant existing at the high temperature.

When moistening in superheated steam, there exists a 60 simple relationship between the temperature of the steam and the moisture ratio of the sheet whereby, as the temperature of the steam increases, the moisture ratio of the sheet decreases. This relationship is diagrammatically illustrated in Fig. 2. The curve of Fig. 2 is somewhat similar to the curves of the hygroscopic properties 65 of selected materials which are available in the "Inter-

national Critical Tables." For example, in the volumes published for the National Research Council by McGraw-Hill Book Company in 1933, such curves appear in volume 2 at pages 321 et seq. These curves plot the moisture ratio of the material against the relative humidity of the surrounding moist air at equilibrium, and it is a simple matter to derive a curve such as shown in Fig. 2 which plots the moisture ratio of the material against the temperature of superheated steam.

With the curve of Fig. 2, the state of the steam (in degrees of superheat or in temperature and pressure) which is in equilibrium with fibreboard having a selected moisture ratio, may be determined. The percentage moisture, which is the weight of moisture divided by the weight of bone dry material is plotted as the ordinate, and the temperature expressed in degrees centigrade is plotted as the abscissa. The curve plots the values for steam at one atmosphere of pressure. Reading from the curve, fibreboard having a moisture ratio of 22% would be in equilibrium with atmospheric steam at 100 degrees centigrade. Atmospheric steam at 104 degrees centigrade would be in equilibrium with fibreboard having a moisture ratio of 0.12 (see point D on the curve). Atmospheric steam at 105 degrees centigrade would be in equilibrium with fibreboard having a moisture ratio of 0.095 (see point E). Atmospheric steam at 110 degrees C. would be in equilibrium with fibreboard having a moisture ratio of 0.07 (see point G). By using the curve of Fig. 2, the state of the steam at atmospheric pressure and any selected temperature may be expressed in terms of the moisture ratio ( $U_v$ ) of the fibreboard in equilibrium therewith. Thus, steam at one atmosphere and 115 degrees C. may be defined as having a  $U_v$  of 0.06 (see point H). At other pressures and temperatures, the  $U_v$  of the steam may still be 0.06, in accordance with the values of the humidifying force of the steam at such pressures and temperatures.

The curve of Fig. 1 illustrates a standard pressing cycle showing the increase in temperature as the pressing cycle progresses. The work sheets are charged into the pressing device at the time O and are exposed to pressure and heat. At time A, the temperature of the sheet reaches a level where the sheets are practically bone dry. The sheets are usually retained in the device until the time B, during which period they are heated to the temperature of the surfaces of the pressing device. In many operations, the procedure is interrupted at the time C and the sheets are heat-treated in a separate device.

When a sheet is discharged from the pressing device, a certain amount of time will elapse before the sheet is transported to the succeeding treatment. During this time, the sheet will cool. If the sheet is exposed to heat treatment, its temperature will be raised to a temperature of about 170 to 200 degrees C. The sheet then can be charged into the moistening apparatus with a temperature of about 150-160 degrees C. When moistening in superheated steam at this temperature, the material must have an equilibrium moisture ratio of about 0.01 to 0.02 or a percentage moisture of about 1 to 2 percent. By moistening, a percentage moisture of about 7% is desired in order to obtain equilibrium with air at normal atmospheric conditions. In order to attain this equilibrium condition, it is necessary to lower the temperature of the steam successively down to about 110 degrees C. (see point G on the curve of Fig. 2). It is possible to proceed with the treatment as indicated in Figs. 3, 3a or 4.

Figs. 3 and 3a illustrate the cycle of moistening in a chamber where the sheets are stationary and the condition of the treating medium is gradually changed stepwise during the treatment period. Fig. 4 shows a cycle in apparatus for continuously moistening sheets. In this case, the sheet is moved countercurrent to a steam cur-

rent, the "relative moisture" or superheating of which is varied with respect to the time. In carrying out the invention, the moistening steps should be controlled so that the state of the steam in terms of the moisture ratio of material in equilibrium with the steam, is gradually varied in relation to the actual moisture ratio of the sheet. This variation is continued until the moisture ratio of the material reaches about  $\frac{1}{2}$  of the intended final moisture ratio of the sheet, for example, as indicated at the time F in Figs. 3, 3a and 4, and then the state of the steam is adjusted so that the moisture ratio of the material in equilibrium with the steam is equal to the desired final moisture ratio of the sheet. In the curves  $U_v$  indicates the state of the steam in terms of the moisture ratio of the material in equilibrium with the steam, and  $U_m$  indicates the actual moisture ratio of the material.  $U_{mf}$  indicates the desired final moisture ratio of the sheet.

Referring to Fig. 3, during the moistening cycle, the  $U_v$  of the steam is gradually increased stepwise as the  $U_m$  of the material increases. If the moistening occurs at atmospheric pressure, the temperature of the steam is gradually reduced. The values for  $U_m$  may be estimated to obtain the curve shown in Fig. 3, or the moistening cycle may be run and test samples taken intermittently to determine the  $U_m$ . When the curves  $U_v$  and  $U_m$  have been determined, it is not necessary to take repeated samples or readings of the  $U_m$ , and the  $U_v$  of the steam may be increased according to the pattern initially determined.

The regulation may also be performed as shown in Fig. 3a in such a manner that the ratio  $U_v/U_m$  is equal to 2-5, preferably about 3. As shown, the  $U_v$  of the steam is changed in steps from 0.01 to 0.12 approximately, which in atmospheric pressure, would mean a temperature variation in steps from about 200 degrees C., down to 104 degrees C., at the time F the  $U_v$  is reduced to the value of  $U_{mf}$ , for example by raising the temperature to 110 degrees C.

Fig. 4 shows the cycle where the state of the steam is changed continuously, for example as when the material travels through a tunnel ranging in temperature from approximately 200 degrees C. down to 110 degrees C.

After the moistening cycle, the sheet has a moisture ratio nearly equal to  $U_{mf}$ . If the sheet is not heat-treated before moistening, for instance during the hardening, it is necessary to heat the sheet to prevent condensation. The sheet should be heated to or above the dew point of the steam used in the moistening. The sheet should preferably be heated to a temperature corresponding to the dry bulb temperature of the steam at the beginning of the moistening to insure against water vapour condensation at the surface of the sheet at the beginning of the moistening.

At the end of the moistening the sheet has a temperature corresponding to the desired equilibrium moisture ratio. When moistening in super-heated steam the sheet will thus reach a temperature of about 110° C. corresponding to a "normal" moisture content of the sheet. If such a warm sheet is directly introduced into a normal room-atmosphere at about 20° C. and 50% relative humidity, the sheet will lose a part of its moisture content while being cooled. In order to prevent this, the sheet should in accordance with the invention be cooled to or near to the room temperature by means of air whose condition is maintained near the equilibrium state intended for the sheet, so that the sheet during its cooling neither gives off nor absorbs moisture from the cooling air. It is also possible to proceed in such a manner that the sheets are moistened somewhat above the normal moisture ratio and then discharged while warm. When the sheets cool, they give off a small part of their water content to the surrounding cool room atmosphere.

Heat treatment (or only heating) and moistening and cooling of the sheets may be performed in apparatus ac-

cording to Fig. 5. The plant principally consists of two chambers 1 and 2 provided with sealed closing doors 3. By means of partition 14 the chambers are divided into a treating space 1b and 2b respectively and a channel 1a and 2a respectively for a circulating medium. In each of the circulating channels there is a fan 4 driven by a motor 5. These fans are intended to circulate the treating medium through the goods (the sheets) 6 piled for instance on trucks. The chamber 1 is furthermore provided with one or more jets 7 for supplying steam into the chamber and also with heating elements 8 for the supply of heat to the sheets and for the super-heating of steam. The supply of moisture to the jets 7 is controlled by a valve 7a, and the heating elements are controlled by a valve 8a. The chamber 2 is provided with jets 9 (controlled by a valve 9a) for steam or water and drop traps 10 for eliminating water drops from the jets. In order to make it possible to exhaust gases generated during the heat treatment (hardening) the chamber 1 is provided with a chimney 11. The chamber 2 is provided with an inlet 12 for air and an outlet 13 for ventilating air, the object of which air is to carry away heat from the sheets during the cooling. The flow of air through the inlet and outlet may be controlled by dampers 16 and 17.

The treatment of the sheets is performed in the following manner. The sheets delivered from the pressing device are piled on a truck charged into the chamber 1. By means of the heating element 8 and the circulating fan 4 the sheets are rapidly heated up to the hardening temperature usually 170-200° C. This temperature is maintained during a certain time often about 3-5 hours. While the sheets still are warm the valve 7a is operated to supply steam through the jet 7, whereby air and gas are forced out from the chamber and caused to escape through the chimney 11. The pressure of the chamber is then regulated by means of a damper 15 arranged in the chimney. The temperature of the super-heated steam is gradually reduced by operating the valve 8a to a value at which the moisture ratio of the sheet in equilibrium therewith corresponds to the moisture ratio intended for the moistened sheet. The reduction in temperature causes the  $U_v$  of the steam to rise, for example, as indicated in Figs. 3, 3a, or 4. When the sheet is moistened it will have a temperature somewhat above 100° C. and the sheet must therefore be cooled before it can be stored. The sheets are for this reason transported to the chamber 2 where they are cooled by air supplied through the duct 12. The used air (having higher water and heat contents than the supplied air) will escape through the duct 13. In order to make it possible to regulate the humidity of the air during the cooling so that the desired moisture ratio is maintained in the sheet, the valve 9a is operated to supply the necessary quantity of moisture through the jet 9. Any water drops are eliminated in the drop trap 10. The sheet can also be cooled by means of cool air without any addition of water, but the moisture which has been added to the sheet in the moistening apparatus will partly be lost.

The heat treatment of the sheets can also be performed under pressure. If the sheets are moistened before being exposed to the relatively high heat treatment-temperature, to a moisture percentage of about 4-15%, the result of the combined influence of moisture, pressure and temperature will be that the fibres of the sheets are converted ("plastified") and that the absorption of moisture as well as the swelling will decrease substantially. Under certain circumstances it will be convenient to let the sheets remain in the pressing device only until they attain the aforementioned moisture ratio and then expose the sheets to the same treatment. Also the quality of the sheets with respect to working them, for example trimming, dressing etc. will be improved as the sheets by this treatment will obtain a more homogeneous plastic-like structure.

The treatment can be carried out in a closed chamber (autoclave) substantially of the design shown in Fig. 6. The apparatus consists of a receptacle 21 constructed to withstand high pressures. In this receptacle there is an inner casing 22 designed to contain a truck 23 on which the sheets to be treated are piled. Said inner casing is on its bottom provided with two rails 24 for the truck. The receptacle 21 is at one of its ends provided with a swinging door 25 where a gas distributing means 26 (for instance a perforated plate) is fastened so that it can follow the movements of the door. The distributing means is adapted to register with the surface of the inner casing 22. In the rear part of the inner casing there is a similar distributing means 27 at some distance from the rear end wall 28 of the inner casing. In the wall 28 there is a central outlet for gaseous medium to which a fan 29 is connected. The fan is driven by means of a shaft 30 passing through the rear wall 35 of the receptacle. For the shaft 30, a packing box 31 is mounted in the wall 35. A channel for circulating medium is formed between the outer and inner casings of the apparatus and in this channel there are heating elements 32 controlled by a valve 36 and a steam inlet 33 controlled by a valve 37. The purpose of the inlet for steam is partly to supply moisture to the sheets (boards) and partly to maintain the pressure in the receptacle.

The treatment is performed in the following manner. The receptacle is charged with a truck with piled sheets to be treated. The sheets are then heated to a temperature equal to or somewhat above the steam temperature at which the sheets obtain the intended moisture ratio. The sheets will reach about 5% of moisture ratio at atmospheric pressure and at a temperature of about 105-110° C. At a super-pressure of 2 atmospheres and with saturated steam in the receptacle the sheets will have a moisture ratio of about 15%. For the conversion (plastifying) of the sheets it is then necessary to raise the temperature and the pressure, as the conversion takes place in the sheets more rapidly at a high pressure and at a high temperature. The maximum temperature which can be used depends on the origin of the cellulose fibres. For fibres of different kinds it is possible to use temperatures between 160-220° C. and super-pressure of about 6-24 atmospheres corresponding to the temperature of the saturated steam. When the conversion has continued to a certain degree the pressure and the temperature is lowered to values corresponding to the moisture ratio of the sheet which is in equilibrium with normal atmospheric conditions. Fig. 7 shows diagrammatically the progress of the temperature and the pressure during a cycle. The invention is of course not limited to the temperatures and pressures illustrated in the figure. The process may be modified within wide limits with respect to the material to be treated.

The moistening and heat treating of the sheets under pressure produces—besides an improved plastic quality, a reduced absorption of moisture and a reduced swelling—the advantage of a shortened pressing time resulting in an increased production by the existing equipment. This is of a great economic importance as the pressing device is more expensive than the heat treating apparatus.

What we claim is:

1. An improved method of treating fibre boards and like materials manufactured by defibrating fibrous raw materials, forming, dehydrating, and drying in a pressing device the dehydrated material, comprising the steps of heat-treating the material up to a temperature of 100-180° C., preferably 150-160° C., subsequently moistening the material while at said temperature by air-free steam, and cooling the material after moistening, said moistening step being performed for at least an initial and major portion of said step by gradually changing the state of the steam in relation to the actual mean-moisture ratio of the material in such a manner that the ratio of  $U_v$  to  $U_m$  is maintained at a substantially constant value

(where  $U_v$  stands for the state of the steam in terms of the moisture ratio of the material which would be in equilibrium with said steam and  $U_m$  is the actual moisture ratio of said material).

2. A method according to claim 1 wherein in said heat-treating step the material is heated to a temperature corresponding to the dry bulb temperature of the steam employed at the start of the moistening step.

3. A method according to claim 1 wherein said cooling step cools the moistened material approximately to room temperature by means of air having a relative humidity and temperature providing a humidifying force equal to the humidifying force of atmospheric air.

4. A method according to claim 1 wherein said heat-treating step comprises heating the material to at least 15 the dew-point of the air-free steam in the moistening step.

5. A method according to claim 4 wherein said ratio of  $U_v/U_m$  is in the range between 2 and 5.

6. A method according to claim 5 wherein said ratio of  $U_v/U_m$  is maintained until the material attains a moisture ratio equal to  $\frac{2}{3}$  of the desired final value and thereafter the state of the steam is maintained constant so as to make  $U_v$  equal to the desired final moisture ratio.

#### References Cited in the file of this patent

##### UNITED STATES PATENTS

|    |            |               |               |
|----|------------|---------------|---------------|
| 10 | Re. 22,071 | Nevin         | Apr. 14, 1942 |
|    | 1,421,685  | Glessner      | July 4, 1922  |
|    | 2,000,663  | Darrah        | May 7, 1935   |
|    | 2,376,612  | Muench et al. | May 22, 1945  |

##### FOREIGN PATENTS

|         |               |                |
|---------|---------------|----------------|
| 335,942 | Great Britain | Oct. 3, 1930   |
| 416,552 | Great Britain | Sept. 17, 1934 |